

July 17, 1962

V. E. VALENTINE

3,044,124

ROTATIONAL CASTING

Original Filed Sept. 5, 1957

3 Sheets-Sheet 1

FIG. 1



July 17, 1962

V. E. VALENTINE

3,044,124

ROTATIONAL CASTING

Original Filed Sept. 5, 1957

3 Sheets-Sheet 2

CHARGING & CLOSING MOLDS

FIG. 3a



FIG. 3



FIG. 3b



NO ROTATION  
TEMP < 130° F

DISTRIBUTION

FIG. 4a



FIG. 4



FIG. 4b



2-30 RPM  
2-5 SEC.

PARTIAL GELLING (THIN LAYER)

FIG. 5a



FIG. 5



FIG. 5b



50-150 RPM  
15-20 SEC.

INVENTOR  
VAUGHN E. VALENTINE

BY

*Hamilton & Cook*

ATTORNEYS

July 17, 1962

V. E. VALENTINE

3,044,124

ROTATIONAL CASTING

Original Filed Sept. 5, 1957

3 Sheets-Sheet 3

FULLY GELLED

FIG. 6α



FIG. 6



SET

FIG. 6α'



FIG. 6'



FIG. 6b



COOLING

FIG. 7α



FIG. 7



FIG. 7b



INVENTOR  
VAUGHN E. VALENTINE

BY *Hamilton & Cook*

ATTORNEYS

1

3,044,124  
ROTATIONAL CASTING

Vaughn E. Valentine, South Hadley, Mass., assignor to The Sun Rubber Company, Barberton, Ohio, a corporation of Ohio  
Original application Sept. 5, 1957, Ser. No. 682,099, now Patent No. 2,957,202, dated Oct. 25, 1960. Divided and this application Aug. 19, 1960, Ser. No. 54,333  
8 Claims. (Cl. 18—58.3)

The present invention relates to improvements in the rotational casting of synthetic resins such as vinyl plastisols and similar materials. More particularly, the invention relates to improved rotational casting methods.

In the rotational casting of intricate articles, e.g. the arms or legs of a play doll, it has been found that conventional techniques are not completely satisfactory. During the early stages of this art, much effort was expended in perfecting apparatus and methods for the casting of even uncomplex shapes such as the play balls or footballs. As this phase was perfected, increasing attention was paid to the problems of casting more intricate shapes. Apparatus then in use was modified in an effort to achieve the desired versatility. However, these efforts have met with only limited success.

Therefore, it is an object of the present invention to provide an improved method for the rotational casting of intricate articles having superior properties and appearance; such invention also being applicable to improved production of relatively uncomplex shaped articles.

Some further objects are: to provide an improved method which involves rotating mold carriers on their "major" and "minor" axes at different speeds and in selective sequence; to provide a more efficient method for simultaneous loading, curing and cooling of a series of molds; and to provide improved casting methods which are performed during the curing and cooling stages to produce an article having superior physical properties and appearance.

These and still other objects of the invention will be apparent in view of the following detailed disclosure including the drawings.

In the drawings:

FIG. 1 is a plan view showing schematically operation of the casting apparatus practicing the method of the invention;

FIG. 2 is a section taken substantially as indicated on line 2—2 of FIG. 1;

FIG. 3 is a schematic representation partly broken away of an individual mold as shown in FIG. 2 depicting the mold charged and closed;

FIG. 3a is an enlarged fragmentary area of FIG. 3;

FIG. 3b is a schematic representation of means for biaxial rotation of the mold shown in FIG. 3;

FIG. 4 is a figure similar to FIG. 3 showing the initial distribution of the plastisol charged within the mold;

FIG. 4a is an enlarged fragmentary area of FIG. 4;

FIG. 4b is a schematic representation of the mold being rotated about one axis;

FIG. 5 is a figure similar to FIG. 3 showing the partial gelation of the plastisol charge within the mold;

FIG. 5a is an enlarged fragmentary area of FIG. 5;

FIG. 5b is a schematic representation of the high speed rotation of the mold about one axis;

FIG. 6 is a figure similar to FIG. 3 showing the plastisol charged within the mold fully gelled;

FIG. 6a is an enlarged fragmentary area of FIG. 6;

FIG. 6' is a figure similar to FIG. 6 showing the plastisol charge within the mold fused, or fully set;

FIG. 6a' is an enlarged fragmentary area of FIG. 6';

FIG. 6b is a schematic representation of the rotation of the mold about dual axes;

2

FIG. 7 is a figure similar to FIG. 3 depicting the plastisol charge within the mold as being completely fused and cooled;

FIG. 7a is an enlarged fragmentary area of FIG. 7;

FIG. 7b is a schematic representation of the mold being rotated about one axis during the cooling stage.

A preferred form of casting apparatus used to practice the method of the invention is shown in the drawing and indicated generally by the numeral 20. A detailed

10 description of the preferred apparatus is disclosed in U.S. Patent No. 2,957,202, issued on the parent application filed on September 5, 1957, in the name of Paul Rekettye and Vaughn E. Valentine, Serial No. 682,099. The mold carriers are indicated generally by the numeral 22.

15 The curing oven is indicated generally by the numeral 24.

In the form of the machine 20 as shown, there are provided three equally spaced (120° apart) mold-carrying arms, indicated generally by the numeral 35. Each arm 35 includes a solid shaft 36 coaxially enclosed within

20 or by a tubular shaft 37. The shaft 36 is driven to rotate the mold carriers 22 on their "major axis." The shaft 37 is driven to rotate the mold carriers on their "minor axis."

25 Selective rotation of shafts 36 and 37 may be controlled

automatically by a clutch assembly (not shown), and the mold carrying arms 35 may be successively rotated

through the stripping and loading (I), the curing (II)

and the cooling (III) stations manually or by an indexing mechanism.

30 After the molds 100 have been charged with a pre-

determined amount of liquid plastisol (FIG. 3), the outer

section 97 is fitted on the shaft 43, a cap 102 is aligned

with each mold 100, and the locking assembly 99 is

tightened.

35 As used herein, the terms "plastisol charge" or "resinous

plastisol" are intended to mean a mixture of synthetic

resin(s) and plasticizers which can be molded, cast or

converted to continuous films by the application of heat.

The term "synthetic resin(s)" is intended to mean a

40 thermoplastic, complex, substantially amorphous organic

semi-solid or solid material (usually a mixture) built

up by chemical reaction of comparatively simple com-

pounds, approximating the natural resins in luster, frac-

ture, comparative brittleness, insolubility in water, fusibil-

45 ity or plasticity, and some degree of rubber-like ex-

tensibility; but commonly deviating widely from natural

resins in chemical constitution and behavior with reagents.

More specifically, the terms include the vinyl polymers

and copolymers such as polyvinyl chloride (P.V.C.).

50 Without in any sense limiting the scope of the invention

to the proportions set forth, the following is a detailed

description of one suitable formula for use in the manufac-

ture of articles according to the invention, the compound

formulation being known as a vinyl plastisol.

55 To 100 parts of a conventional polyvinyl chloride

polymer, such as is well known to those skilled in the

art, for example, the compound Geon 121, obtainable

from the B. F. Goodrich Chemical Co., is added: 80

parts of a conventional plasticizer, such as di-(2-ethyl-

60 hexyl) phthalate (DOP), also well known to those skilled

in the art; 2 to 6 parts of a liquid barium-cadmium sta-

bilizer; such as Advastab X23-30 obtainable from the

Advance Solvents & Chemicals Corp., also well known

to those skilled in the art, and inert pigment as re-

quired depending upon the color desired for the plastisol.

A plastisol having this formulation gels at about 130° F.,

fuses at about 340° F. and chars at about 370° F.

(maintained in excess of 5 minutes). This mixture is

90 schematically depicted in FIG. 3, and the enlarged area

depicted by FIG. 3a, to show the resin particles suspended

in the liquid plasticizer. Such fragmentary areas are

shown for each of the figures representing the process to

schematically depict the well-known increase of colloidal substance as the resin and plasticizer solvates during distribution, gelation and fusion. A more complete discussion of the gelling and fusion of plastisols is given in U.S. Patent No. 2,629,134 to Molitor.

At the loading and stripping station (I), shafts 36 and 37 are stationary and the molds 100 are cooled to substantially room temperature, in any event less than 130° F. After the molds are charged, with a predetermined amount of plastisol, and closed, the casting machine turret is rotated toward the curing oven 24.

The temperature of the oven 24 is so chosen as to provide sufficient heat energy to bring the walls of the cool molds up to the fusing temperature within the time allotted for the curing cycle. The exact temperature at which the oven is maintained will depend upon the oven insulation, the thickness and heat transfer rate of the mold walls, the size of the oven doors 105, and other factors. Selection of the proper oven temperature is within the knowledge of those skilled in this art.

As the arm 35 enters the oven, shaft 37 is rotating at a rate selected from the range 2-30 r.p.m. Such rotation on the "minor axis" is of brief duration (2 to 5 seconds) and causes full distribution of the plastisol in the remote and intricate areas of the molds 100 (see FIGS. 4, 4a and 4b). Of course, to accomplish this in the embodiment shown, the "minor axis" must be parallel to the ground. Such rotation also ensures that the cool molds will be heated at a uniform rate with no localized areas having significant temperature differences.

Substantially simultaneously with the indexing of arm 35 at curing station (II), and with the "minor axis" maintained parallel to the ground, shaft 37 is spun at a rate selected from the range 50-150 r.p.m. (FIGS. 5-5b). Such high speed rotation on the minor axis is of longer duration (15 to 20 seconds) and continues until a very thin gelled layer of plastisol is formed on the walls of the mold. It has been found that the centrifugal force generated by the high speed rotation, while heating the mold so that the outermost layer of plastisol is gelled, will be sufficient to cause the plastisol to remain in the remote and intricate areas of the mold during the final curing and solidifying stages of the process.

Before the plastisol has gelled beyond the thin outer layer, the high speed rotation is stopped, and simultaneous rotation on both axes at a rate selected from the range 2-30 r.p.m. takes place for a period of about seven minutes, or until the plastisol has fully gelled (FIG. 6) and set (FIG. 6'). After the plastisol charge has fused, the arm 35 which has been in the furnace, is indexed to the cooling station.

At the cooling station (III), the "minor axis" shaft 37 only is rotated (see FIG. 7) and the mold carriers 22 are first immersed in a water bath 108. The temperature of the bath 108 is approximately 150° F. and the molds are rotated therein for approximately 30 seconds. The temperature of the bath and the duration of rotation therein are so chosen as to ensure that the solidified plastisol is quickly lowered to a temperature significantly below the setting temperature, so that there can be no deterioration of the product. After immersion cooling in the bath, the mold carriers are further cooled by slow rotation in air for the balance of the cycle (7 minutes or less). At the end of the cooling period, the temperature of the products within the mold should be 120-130° F.

Specific operating times and temperature for a specific vinyl plastisol formulation, have been described. It will be apparent however, that minor changes could be made therein without departing from the basic concepts of the invention. Accordingly, the scope of the invention should be determined by the fairly implied scope of the joined claims.

What is claimed is:

1. In a process for casting intricate hollow articles from a vinyl resin plastisol, said process requiring a heating

zone at the curing temperature of said plastisol, the steps of, locating a series of molds radially of a first axis and transversely to a second axis, charging said molds when at a temperature below 130° F. with a predetermined amount of plastisol, closing said molds, introducing said closed molds into said heating zone while rotating the molds at from 2-30 r.p.m. on said first axis, rotating said molds at from 50-150 r.p.m. on said first axis as the temperature of the molds rises to the gelling temperature of said plastisol, and, before the plastisol has gelled beyond a thin outer layer, simultaneously rotating the molds at rates of from 2-30 r.p.m. on both axes as the temperature of the molds rises to the fusing temperature of the plastisol.

5 2. In a process according to claim 1, the additional steps of rapidly lowering the temperature of said molds to below the fusing temperature of said plastisol while rotating said molds at from 2-30 r.p.m. on said first axis, gradually lowering the temperature of said molds to a temperature below 130° F., and opening said cooled molds and removing the articles.

10 3. In a process for casting intricate hollow articles from a synthetic resin plastisol, said process requiring a heating zone at the curing temperature of said plastisol, the steps of, locating a series of molds radially of a first axis and transversely to a second axis, charging said molds when outside said heating zone with a predetermined amount of plastisol, closing said molds, introducing said closed molds into said heating zone while rotating the molds at a slow rate on said first axis, rotating the molds at a high rate on said first axis as the temperature of the molds rises to the gelling temperature of said plastisol, and, before the plastisol has gelled beyond a thin outer layer, simultaneously rotating the molds at a slow rate on both axes as the temperature of the molds rises to the fusing temperature of said plastisol.

15 4. In a process according to claim 3, the additional steps of rapidly lowering the temperature of said molds to below the fusing temperature of said plastisol while rotating said molds at a slow rate on said first axis, gradually lowering the temperature of said molds to a temperature below 130° F., and opening said cooled molds and removing the articles.

20 5. In a process for casting intricate hollow articles from synthetic resin plastisols, the steps of charging a cool mold with a predetermined amount of plastisol, closing the mold, distributing the plastisol in those portions of the mold forming the intricate portions of the article, subjecting said closed mold to strong centrifugal forces of rotation on a first axis while raising the temperature of the mold to the gelling temperature of said plastisol, and, before the plastisol has gelled beyond a thin outer layer, further subjecting said mold to simultaneously applied weaker rotative forces on said first axis and on a second axis divergent therefrom while raising the temperature of the mold to the fusing temperature of said plastisol.

25 6. In a process according to claim 5, the additional steps of rapidly lowering the temperature of said molds to below the fusing temperature of said plastisol while rotating said molds at a slow rate on said first axis, gradually lowering the temperature of said molds to a temperature below 130° F., and, opening said cooled molds and removing the articles.

30 7. In a process for casting intricate hollow articles from synthetic resin plastisols, the steps of charging a mold with a predetermined amount of plastisol, closing the mold, distributing the plastisol in those portions of the mold forming the intricate portions of the article, subjecting said closed mold to a strong centrifugal force on a single axis while raising the temperature of the mold to the gelling temperature of said plastisol, and before the plastisol has gelled beyond a thin outer layer, further subjecting said mold to simultaneously applied weaker rotative forces having divergent axes while raising the

temperature of the mold to the fusing temperature of said plastisol.

8. For rotational casting of synthetic resin plastisols, a process including the steps of, exposing a closed mold charged with a predetermined amount of plastisol to heat sufficient to gel the layer of plastisol in contact with the interior of said mold while the mold is subjected to slow rotation and then strong centrifugal forces on a single axis, further heating said mold to a temperature sufficient to fuse said plastisol while said mold is subjected to a plurality of rotative forces having divergent axes, and rapidly lowering the temperature of said mold to below the fus-

ing temperature of said mold while the mold is subjected to weaker centrifugal forces on said single axis.

References Cited in the file of this patent

UNITED STATES PATENTS

|   |           |                  |       |               |
|---|-----------|------------------|-------|---------------|
| 5 | 2,659,107 | De Bell          | ----- | Nov. 17, 1953 |
|   | 2,834,986 | Bailey et al.    | ----- | May 20, 1958  |
|   | 2,958,907 | Mumford et al.   | ----- | Nov. 8, 1960  |
|   | 2,967,329 | Friedland et al. | ----- | Jan. 10, 1961 |

10

OTHER REFERENCES

"Rotational Casting of Plastisols," from Modern Plastics, September 1954, 4 pages.